

Nov. 13, 1973

G. THOMAS ET AL

3,772,415

PROCESS FOR PREPARING YARN PACKAGES

Filed Dec. 13, 1971

FIG.1



FIG.2



**1**

3,772,415

**PROCESS FOR PREPARING YARN PACKAGES**  
Gwylfa Thomas and Brian William Jenkins, Pontypool,  
England, assignors to Imperial Chemical Industries  
Limited, London, England

Filed Dec. 13, 1971, Ser. No. 207,247

Claims priority, application Great Britain, Dec. 16, 1970,  
59,716/70

Int. Cl. B29c 25/00

U.S. Cl. 264—234

4 Claims

**ABSTRACT OF THE DISCLOSURE**

Process and apparatus for minimising the variation in through package retraction that occurs in packages of freshly drawn thermoplastic yarn by heating the yarn after drawing according to a defined programme.

The present invention relates to retraction uniformity in yarn packages and particularly though not exclusively to a process and apparatus for achieving such uniformity.

Conventionally, and in order that (mono- or multi-filament) yarns derived from synthetic thermoplastic polymers such as polyamides and polyesters may be usefully employed in normal textile operations, they must be molecularly orientated or stretched (drawn) after extrusion and solidification from the molten polymer. The drawing process may be conveniently carried out by passing the yarn sequentially around two rolls which are rotated at different speeds, thus, if the second roll (draw roll) is rotated, say, at three times the speed of the first (feed roll), the yarn will be stretched by that amount between them. Finally, the drawn yarn, usually under some degree of relaxation, is wound either directly or indirectly on to a bobbin by, say, a ring and traveller assembly which simultaneously inserts a small amount of stabilising twist into the yarn.

Freshly drawn yarn, however, though wound on to a bobbin is still tending to shrink and in these circumstances a situation somewhat akin to the following arises. The innermost package layers because they are held firmly against the container barrel are unable to shrink, while the outer package layers shrink to some extent onto the layers beneath. The middle package layers are less free to shrink and are subjected to crushing due to the shrinkage of the outer layers. Thus, when yarn is taken from the package, the residual tendency to shrink or retract is lowest in yarn from the middle of the package and greatest in yarn from the inside.

In practice this variation in retraction manifests itself as an undesirable variation of dye up-take (stripiness) in a final woven or knitted fabric, and arises not only from a variation of retraction through a single yarn package, but from the "jump" in retraction that occurs when yarn from one package is joined to yarn from another, as in magazine creeling, since it is yarn from the inside of one package that is joined to yarn from the outside of another.

In the present invention the applicants have sought to minimise this variation in retraction in freshly drawn yarn packages by heating the freshly drawn yarn in a defined manner before winding up.

Thus, the present invention provides a process for minimising the variation in through package retraction that occurs in packages of freshly drawn thermoplastic yarn in which the yarn after drawing and prior to being wound onto a bobbin is heated to gradually decreasing temperatures until a minimum temperature is reached and thereafter is heated to gradually increasing temperatures, the changes in temperature corresponding to the substantial changes in retraction that would otherwise occur through the package.

**2**

The present invention also provides a thermoplastic yarn drawing apparatus for carrying out the above process in which variable heating means are located between the draw roll and yarn wind up means.

Roughly speaking, the gradual decreasing and increasing yarn temperature occurs, respectively, during the winding of the first and final "thirds" of the yarn package.

Besides minimising variation in through package retraction, the process and apparatus of the present invention also reduce the overall level of retraction that occurs in freshly drawn yarn. Thus, although directed to the reduction of variation in through package retraction, the practice of the present invention results in an overall reduction in the magnitude of any residual retractive forces that might arise in packages of freshly drawn yarn.

One convenient way of heating the freshly drawn yarn according to the present invention is to locate the heating means in the form of an electrically heated pin or plate immediately after the draw roll in the drawing process, though the heating device may be located further downstream of the draw roll should such an arrangement prove attractive in terms of apparatus geometry.

The applicants prefer to use a 4 inch diameter heated matt chrome pin located immediately after the draw roll.

In the following example of the present invention which is by way of illustration only, a 40 denier 13 filament yarn derived from polyhexamethylene adipamide was drawn at 2,646 f.p.m. and passed around a 4 inch diameter heated matt chrome pin located immediately after the draw roll in a conventional drawtwister machine. The yarn was wound up with a ring and traveller assembly at constant spindle speed to form a 32 oz. multi-cycle yarn package.

During the winding of approximately the first 10 ozs. of yarn, the temperature of the heated pin was gradually decreased from 150° C. to 70° C., and then after approximately 20 ozs. of yarn had been wound the temperature of the pin was gradually increased to 150° C. again at 32 ozs.

FIGS. 1 and 2 show respectively, according to the above example, the change in pin temperature and the change in percentage yarn retraction with increasing package weight. It will be apparent that each unit length of yarn is heated to essentially one temperature which is different for each unit length.

In FIG. 2, for comparative purposes, the change in percentage yarn retraction when a heated pin was not employed is shown at A.

Yarn retraction is defined as the reduction in length which occurs in yarn suspended vertically under a stress of 0.002 to 0.007 gm./d. in air over a period of at least 24 hours. In the present invention retraction was determined by cutting a measured length of yarn (1.5 metres) from a threadline at a tension of 0.005 to 0.05 gm./d. running at a speed of 5 m./sec., and freely suspending this length under a weight corresponding to 0.002 gm./d. for the required period. Retraction is then expressed as a percentage change of the original cut length. Prior to the determination the yarn package to be tested was conditioned for at least 24 hours in the atmosphere in which the test was conducted, i.e. in air at 18° C.—27° C. and 59%—71% relative humidity.

When knitted fabrics comprising yarn of the above example were dyed with Chlorazol violet or Solway blue BN, no stripiness due to yarn retraction variations was visible. In similar fabrics comprising untreated yarns, stripes were clearly visible after dyeing.

What is claimed is:

1. In a process for drawing and winding polyamide yarn onto a bobbin to form a package, the improvement which minimizes the variation in through package retrac-

tion that occurs in packages of freshly drawn yarn, said improvement comprising after drawing and prior to winding the yarn heating the yarn by heating means, decreasing the temperature of the heating means during winding to a minimum temperature and thereafter increasing the temperature again before winding is completed, the changes in temperature corresponding to the substantial changes in retraction that would otherwise occur through the package.

2. A process according to claim 1 in which a gradual decreasing and increasing of the temperature of the heating means occurs respectively during the winding of the first and final thirds of the yarn package.

3. A process according to claim 1 in which the yarn is wound onto a bobbin rotated at constant speed.

4. In a process for drawing and winding polyamide yarn onto a bobbin to form a package, the improvement which minimizes the variation in through package retraction that occurs in packages of freshly drawn yarn, said improvement comprising after drawing and prior to winding the yarn continuously heating the running yarn to a gradually decreasing temperature during winding of about the first one-third of the package and thereafter gradually

increasing the temperature of the running yarn during winding of about the final one-third of the package.

References Cited

UNITED STATES PATENTS

|    |           |         |                  |       |         |
|----|-----------|---------|------------------|-------|---------|
| 5  | 2,794,700 | 6/1957  | Cheney           | ----- | 264—346 |
|    | 2,952,033 | 9/1960  | Goodwin          | ----- | 264—346 |
|    | 3,067,563 | 12/1962 | Dijk             | ----- | 28—62   |
|    | 3,399,108 | 8/1968  | Olson            | ----- | 264—171 |
| 10 | 3,479,426 | 11/1969 | Smedf            | ----- | 264—289 |
|    | 3,547,748 | 12/1970 | D'Onofrio et al. | ----- | 264—346 |
|    | 3,561,082 | 2/1971  | Stanley          | ----- | 264—346 |
|    | 3,618,305 | 11/1971 | Hilbert          | ----- | 28—62   |

FOREIGN PATENTS

|    |        |        |       |       |          |
|----|--------|--------|-------|-------|----------|
| 15 | 10,763 | 4/1970 | Japan | ----- | 28—72.17 |
|----|--------|--------|-------|-------|----------|

JAY H. WOO, Primary Examiner

20 U.S. Cl. X.R.

28—71.3; 242—18 R; 264—210 F, 290 N, 345